



fixed recording layer with a softening or swelling agent for the binder, occasionally in combination with a wetting agent that improves the penetrating power of the hydrophilizing agent in the recording layer. In this way much more zinc oxide grains are reached by the hydrophilizing agent and thus hydrophilized.

As swelling agents preferably water-miscible compounds such as acetone and methyl ethyl ketone are used.

In order to set free zinc ions from the zinc oxide photoconductor, the pH of the hydrophilizing liquid preferably varies between 3 and 6.

According to a preferred embodiment the electrophotographic recording layer is rendered water-receptive at the areas to be hydrophilized after the printing master has been mounted on the press, thus avoiding any separate immersion treatment. The hydrophilizing treatment of the said layer may be carried out by means of an absorbent pad impregnated with an aqueous solution containing the ester compound.

In order to improve the reproducibility of the printing quality, the partially esterified oxy acid compounds of phosphorus are added to the aqueous phase, which is applied during printing separately or together with the lipophilic phase of a planographic printing ink. Thus, e.g. these ester compounds can be added to the aqueous liquid, which is supplied by the damping system to the planographic plate; or can be incorporated into the emulsified aqueous phase of a planographic emulsion type ink.

Electrophotographic recording materials especially suited for use in the preparation of a planographic printing plate are e.g. described in the published Dutch patent applications Nos. 6608814 and 6608815.

Any known process for forming the electrostatic latent image and hydrophobic image can be used.

According to a common technique the hydrophobic image is formed by the subsequent steps of producing an electrostatic image on a photoconductive zinc oxide/hydrophobic binder layer by integrally electrostatically charging that layer, then image-wise exposing and developing the latter layer with a hydrophobic developer powder, which is fixed to the recording layer e.g. by heating.

The powder image can be formed by the known dry "carrier-toner development" or by a liquid development based on electrophoresis wherein charged hydrophobic particles are attracted from an electrically insulating liquid to the charged areas of the recording layer. Such development technique is e.g. described in the U.K. patent specification 755,486.

According to a developing technique described in the United Kingdom patent specifications 987,766; 1,020,505; 1,020,503; 1,033,419 and 1,033,420 an aqueous liquid is image-wise applied to an electrostatic charge pattern present in a recording layer containing photoconductive zinc oxide. Said aqueous liquid can be an aqueous dispersion of hydrophobic material, which after evaporation of the aqueous liquid forms a hydrophobic deposit in accordance with the printing parts.

The following examples illustrate the present invention without, however, limiting it thereto.

#### EXAMPLE 1

A layer of photoconductive material consisting of photoconductive zinc oxide dispersed in an insulating binder (3 parts by weight of zinc oxide to one part by weight of resin binder) was coated on a sheet of aluminum foil laminated to a paper support. The resin binder contained on a weight basis 80% of styrene-butadiene copolymer (80/20), 20% of silicone resin (Silicone resin SR-82 supplied by General Electric-Silicone Products Department, Waterford, N.Y., U.S.A.). The recording layer was charged with a negative corona with a tension of -6000 v. on the corona wires and exposed through a graphic original. Development was carried out by using the magnetic brush technique with iron particles as carrier and gilsonite as fusible toner. The powder image was fixed to the layer by heating for 90 seconds at 140° C.

A cotton pad was impregnated with a solution containing the following ingredients:

|             | Cc. |
|-------------|-----|
| Phytic acid | 10  |
| Water       | 90  |

The plate was rubbed slightly with the cotton pad while on the press. The quality of the prints obtained was very good.

When using 0.3% by weight of phytic acid in the liquid of a damping system of a planographic printing device, up to 5000 excellent sharp copies were obtained.

#### EXAMPLE 2

Example 1 was repeated, with the proviso, however, that the ester compound No. 1 of the table was used. The quality of the plate was fully equivalent to that of Example 1.

#### EXAMPLE 3

A layer of photoconductive material consisting of photoconductive zinc oxide dispersed in an insulating binder (6 parts by weight of zinc oxide to one part by weight of binder) was coated on a flexible aluminum foil.

The binder was prepared from a mixture of EPOK X-1772 (ammoniacal alkyd resin salt marketed as a 66 to 68% (by weight) aqueous solution by British Resin Products) and EPOK W-9801 (a 72% to 75% aqueous solution of a melamineformaldehyde resin marketed by British Resin Products). The coated layer was dried for 24 h. at room temperature and cured for 1 min. at 100° C.

The cured recording layer was charged with a negative corona with a tension of -6000 v. on the corona-wires and exposed to a line-copy.

The electrostatic image was electrophoretically developed by means of an electrophoretic developer prepared by diluting the hereinafter described concentrated developer composition in a ratio of 15/1000 by means of the hydrocarbon solvent Shellsol T (trade name):

Carbon black (average particle size: 20 m $\mu$ ): 30 g.

Zinc tridecyl phosphate (dispersing agent): 1.5 g.

Shellsol T (trade name): 750 ccs.

Resin solution prepared as described hereinafter: 150 g.

The resin solution was prepared by heating at 60° C. 500 g. of Alkydal L 67 (trade name of Farbenfabriken Bayer AG, Leverkusen, W. Germany, for a linseed oil (67% by weight) modified alkyd resin) and 500 ccs. of white spirit containing 11% by weight of aromatic compounds, till a clear solution was obtained.

Hydrophilization of the developed plate was carried out as described in Example 1. When printing with a fatty lithographic ink very sharp prints were obtained.

#### EXAMPLE 4

A layer of photoconductive material consisting of photoconductive zinc oxide dispersed in a ratio of 8 to 1% by weight in an alkyd resin as binding agent was coated on a baryta-coated paper of 135 g./m.<sup>2</sup>. Said recording layer was used for the powder development described in Example 1 and for the electrophoretic development described in Example 3. Hydrophilization after development was carried out as described in Example 1. With the obtained planographic printing master 500 high quality prints were produced.

What we claim is:

1. In a process for preparing a planographic printing plate comprising the steps of forming a latent electrostatic image on a photoconductive insulating recording layer containing an inorganic photoconductive zinc oxide, developing said image with a toner forming a hydrophobic deposit on the image areas of said layer, the improvement of treating the portions of the recording layer which are not covered with said hydrophobic deposit with an aqueous solution containing an oxy acid of phosphorus partially esterified with a polyhydroxy lower aliphatic com-

2. Process for preparing a planographic printing plate according to claim 1, wherein said oxy acid of phosphorus is orthophosphoric acid or pyrophosphoric acid.

3. Process for preparing a planographic printing plate according to claim 1, wherein the said ester is applied to the printing plate after mounting the printing plate on a printing press.

4. Process for preparing a planographic printing plate according to claim 3, wherein the said ester is applied in the aqueous liquid of a damping system of a planographic printing device.

5. Process for preparing a planographic printing plate according to claim 3, wherein the said ester is applied in the aqueous phase of a planographic printing ink composed of a lipophilic phase dispersed in a hydrophilic phase.

6. Process for preparing a planographic printing plate according to claim 1, wherein the said ester is used in

dissolved form in an aqueous liquid in a concentration of 1 to 25 g. per liter.

7. Process for preparing a planographic printing plate according to claim 1, wherein said aqueous solution has a pH of about 3-6.

#### References Cited

##### UNITED STATES PATENTS

|           |        |                    |        |
|-----------|--------|--------------------|--------|
| 3,307,951 | 3/1967 | Adams et al. ----- | 96—33X |
| 3,315,599 | 4/1967 | Lind -----         | 96—1X  |
| 3,323,451 | 6/1967 | Casey et al. ----- | 96—33X |
| 3,386,850 | 6/1968 | Adams et al. ----- | 96—33X |

GEORGE F. LESMES, Primary Examiner

R. E. MARTIN, Assistant Examiner

U.S. CL. X.R.

96—33; 101—465